

[54] **SEPARATION OF MICA FROM CLAY BY FROTH FLOTATION**

[75] Inventor: **David C. Yang**, Edison, N.J.

[73] Assignee: **Engelhard Minerals & Chemicals Corporation**, Woodbridge, N.J.

[22] Filed: **June 26, 1972**

[21] Appl. No.: **266,159**

[52] U.S. Cl. .... **209/166, 252/61**

[51] Int. Cl. .... **B03d 1/02**

[58] Field of Search .... **209/166, 5; 252/61; 106/288 I**

[56] **References Cited**

UNITED STATES PATENTS

|           |         |                 |            |
|-----------|---------|-----------------|------------|
| 2,162,494 | 6/1939  | Trotten .....   | 209/166    |
| 2,759,962 | 8/1956  | Zenftnan .....  | 209/166 UX |
| 3,009,570 | 11/1961 | Lancaster ..... | 209/5      |

|           |         |                   |           |
|-----------|---------|-------------------|-----------|
| 3,037,627 | 6/1962  | Nazen .....       | 209/167 X |
| 3,259,237 | 7/1966  | Scheld .....      | 209/166 X |
| 3,329,265 | 7/1967  | Browning .....    | 209/166   |
| 3,462,013 | 8/1969  | Mencade .....     | 209/166 X |
| 3,480,143 | 11/1969 | Mitzwajer .....   | 209/166   |
| 3,567,636 | 3/1971  | Katzenstein ..... | 252/32 J  |

FOREIGN PATENTS OR APPLICATIONS

|           |         |               |         |
|-----------|---------|---------------|---------|
| 1,044,733 | 11/1958 | Germany ..... | 209/166 |
|-----------|---------|---------------|---------|

Primary Examiner—Robert Halper

Attorney, Agent, or Firm—Melvin C. Flint; Inez L. Moselle

[57] **ABSTRACT**

Mica, present as an impurity in kaolin clay, is removed from the clay by froth flotation in an alkaline pulp with a complex phosphate ester of a nonionic surfactant of the ethylene oxide-adduct type, using an aluminum salt to activate the flotation of the mica.

**5 Claims, No Drawings**

# SEPARATION OF MICA FROM CLAY BY FROTH FLOTATION

## BACKGROUND OF THE INVENTION

High purity kaolin clay is widely used as a coating pigment for paper and paints. Such pigments must be free from abrasive impurities, of which mica is an example. The presence of mica in more than trace quantity may render the clay unsatisfactory for use as a pigment.

Mica can be removed from clay with reasonable ease by gravimetric means or flotation when the clay is coarse. However, when the clay particles and micaeuous impurities are fine, the separation is very difficult. Froth flotation with conventional ionic collectors is usually unsuccessful because mica and kaolin, both silicate minerals, have similar flotation properties.

## THE INVENTION

An object of the invention is to provide a novel method for removing finely divided mica from finely divided kaolin clay by froth flotation.

A specific object is to provide a novel collector system for floating mica from kaolin clay.

Briefly stated, in accordance with the present invention, a micaceous impurity, especially muscovite mica, is removed from kaolin clay by deflocculating a pulp of the impure clay, preferably activating the mica with an aluminum salt, and subjecting the ore pulp to froth flotation in an alkaline flotation circuit in the presence of a complex phosphate ester, or salt thereof, of a non-ionic surface active ethylene or propylene oxide adduct.

## PRIOR ART

Various combinations of anionic and cationic reagents have been suggested as flotation collectors for micaceous minerals. Reference is made to the following patents: U. S. Pat. No. 3,214,018 to Neal; U. S. Pat. No. 3,278,028 to Milsap et al.; U. S. Pat. No. 3,329,265 to Browning et al.

U. S. Pat. No. 2,249,569 to Philips suggests the flotation of kaolin clay from impurities, of which mica is mentioned as an example, by frothing a slip of impure clay with sulfite waste liquor.

## DETAILED DESCRIPTION

In putting the invention into practice, the impure clay ore is blunged in water. Coarse grit and undispersible agglomerates are removed in conventional manner, e.g., by sedimentation, or by treatment in sand boxes.

A clay dispersant (deflocculant) is added before or after degritting. The dispersant used may vary with the nature of the clay. Examples of dispersants are soda ash, sodium silicate, sodium lignosulfonate and sodium condensed phosphates, alone or in combination. Good results have been realized when soda ash was added to adjust pH to a value within the range of 9 to 11 and sodium silicate, phosphate or lignosulfonate was added to deflocculate the pulp and depress the clay.

Water soluble aluminum salts, e.g., aluminum chloride, nitrate or sulfate, are used in carrying out the invention in order to activate the mica. The salts are added as aqueous solutions to the deflocculated alkaline pulps and mixed therewith before adding the collector. Small quantities of aluminum salts are used,

e.b.,  $\frac{1}{4}$  to 1 lb./ton, usually  $\frac{1}{2}$  lb./ton. The aluminum salt can be incorporated into the pulp before or after the phosphate ester collector is added.

The phosphate esters of nonionic surface active agents which are used as collectors in carrying out the invention are described in U. S. Pat. No. 3,567,636 to Katzenstein. The pertinent disclosures in the Katzenstein patent as to the composition of such esters and to their preparation are incorporated herein by reference. Briefly, these are complex phosphate esters (or salt thereof) of a nonionic surface active compound, the phosphate being selected from the group consisting of monoesters, diesters and mixtures thereof, the nonionic surface active compound being the condensation product of an organic hydroxy compound of from 8 to 50 carbon atoms selected from the group consisting of alkyl phenol and alkanols with at least 1 mole of an alkylene oxide having from 2 to 3 carbon atoms, the non-ionic surface active compound containing a maximum of about 50 percent by weight of alkylene oxide based on the weight of the nonionic surface active compound.

The phosphate esters are commercially available under the trade name "GAFAC" and are anionic surfactants. The commercial products are usually mixtures of mono- and di-esters. The product "GAFAC RO-310" is understood to be a mixture of monoester and diester, principally diester. The monoester constituent may be described by the formula:



wherein  $R$  = oleyl; and  $n$  is 4 to 5.

The diester constituent has the formula:



wherein  $R$  = oleyl,  $n$  is 4 to 5.

Obviously the ester can be used in salt form (e.g., sodium, ammonium, calcium, magnesium). In use the acid would be converted to alkali metal salt form in the basic clay pulp.

Generally, the ester is used in amount within the range of 0.1 to 3 lbs./ton, usually within the range of about 0.5 to 1.5 lb./ton.

The phosphate esters normally provide adequate frothing. In some cases, a small amount of a conventional frother such as methyl isobutyl carbinol or pine oil may be added to improve the froth.

Flootation may be carried out at solids within the range of about 5 percent to 50 percent, preferably 20 percent to 45 percent solids.

After flotation the clay in the tailings may be fractionated in conventional manner to recover one or more fine size fractions of beneficiated clay. In some cases, the fine fractions are lower in mica than the flotation tailings.

The following example is given for illustrative purposes and is not to be considered as limiting upon the invention.

The clay used in the test was a kaolin from France. The principal impurity in the clay was muscovite. The degritted minus 325 mesh (Tyler) portion of the impure clay analyzed 2.67 percent  $K_2O$ , corresponding to 22.6 percent muscovite.

A sample of the crude clay (9,000 gm., dry basis) was blunged in deionized water at about 35 percent solids for 15 minutes. The slip was screened on a Sweco vibratory screen and the minus 325 mesh fraction of the slip was recovered.

The degritted slip (minus 325 mesh fraction) was charged to a Fagergren conditioner at 20 percent solids. Soda ash was added in amount of 1.0 lb./ton and the slip was conditioned for 1 minute. The pH was 11.0. Sodium lignin sulfonate was added in amount of 0.5 lb./ton, followed by conditioning for 6 minutes. Aluminum chloride was added in amount of 0.5 lb./ton (calculated as  $AlCl_3 \cdot 6H_2O$ ), followed by 2 minutes' conditioning. GAFAC RO-310, 0.5 lb./ton, was incorporated, followed by 6 minutes' conditioning. The pH of the conditioned pulp was 11.0.

The conditioned pulp was transferred to a Denver flotation machine and the froth was collected. The froth (mica concentrate) and tailings (purified kaolin) were recovered and analyzed. Results are summarized in table form.

Metallurgical results in the table show that froth flotation of the pulp of the impure clay with a phosphate ester complex as the collector reduced the mica content of the clay from 22.6 percent to 12.3 percent at a clay recovery of about 62 percent.

#### FLOTATION OF MUSCOVITE FROM KAOLIN WITH COMPLEX PHOSPHATE ESTER COLLECTOR

| Flotation Product | Wt. % | % $K_2O$ | Muscovite Mica, % | Distribution of Mica, % |
|-------------------|-------|----------|-------------------|-------------------------|
| Head              | 100.0 | 2.67     | 22.6              | 100.0                   |
| Froth Product     | 37.8  | 4.67 *   | 39.6 *            | 66.2 *                  |
| Tailings          | 62.2  | 1.45     | 12.3              | 33.8                    |

\* = Calculated

I claim:

1. In a process for removing a micaceous impurity from kaolin clay, the step comprising subjecting an aqueous alkaline pulp containing kaolin clay and micaceous impurity to froth flotation in the presence of an aluminum salt and a complex phosphate ester, or salt thereof, of a nonionic surface active alkylene oxide adduct as a collector for the micaceous impurity, said phosphate ester being selected from the group consisting of monoester, diester and mixtures thereof, said

nonionic alkylene oxide adduct being the condensation product of an organic hydroxy compound containing from 8 to 50 carbon atoms and selected from the group consisting of alkyl phenol and alkanol with at least 1 mole of an alkylene oxide having 2 to 3 carbon atoms, said nonionic alkylene oxide adduct containing a maximum of about 50% by weight of alkylene oxide.

2. The process of claim 1 wherein said aluminum salt is added to the pulp before adding said complex phosphate ester.

3. The process of claim 2 wherein the flotation is carried out at a pH within the range of 9 to 11.

4. In a process for removing a muscovite impurity from kaolin clay, the step comprising providing a deflocculated aqueous pulp of kaolin clay containing muscovite as an impurity, conditioning said pulp with a water-soluble aluminum salt and thereafter with a small amount of a complex phosphate ester, or salt thereof, of a nonionic surface active ethylene oxide adduct as a collector for the muscovite, and subjecting the pulp to froth flotation, thereby producing a froth which is a concentrate of muscovite and a tailing containing purified clay, said phosphate ester being selected from the group consisting of monoester, diester and mixtures thereof, said nonionic ethylene oxide adduct being the condensation product of an organic hydroxy compound containing from 8 to 50 carbon atoms and selected from the group consisting of alkyl phenol and alkanol with at least one mole of ethylene oxide, said ethylene oxide adduct containing a maximum of about 50% by weight of ethylene oxide.

5. The process of claim 4 in which said phosphate ester is a mixture of monoester and diester, principally diester, wherein the monoester has the following formula:



wherein R = oleyl; and n is 4 to 5; and the diester has the following formula:



wherein R = oleyl; and n is 4 to 5.

\* \* \* \* \*